

W. L. ZIEGLER.  
FLOTATION APPARATUS AND PROCESS.  
APPLICATION FILED APR. 4, 1917.

1,324,139.

Patented Dec. 9, 1919.

Fig. 2.



Inventor

W. L. Ziegler

By  
Mauro Cameron Lewis & Hassie

Attorneys

# UNITED STATES PATENT OFFICE.

WILLIAM L. ZIEGLER, OF SUNSET, IDAHO.

## FLOTATION APPARATUS AND PROCESS.

1,324,139.

Specification of Letters Patent.

Patented Dec. 9, 1919.

Application filed April 4, 1917. Serial No. 159,760.

*To all whom it may concern:*

Be it known that I, WILLIAM L. ZIEGLER, a citizen of the United States of America, and a resident of Sunset, Idaho, have invented 5 a new and useful Improvement in Flotation Apparatus and Processes, which invention is fully set forth in the following specification.

This invention relates to an apparatus and 10 process for the separation of the commingled ingredients of ore material, and is especially adapted for the separation of valuable metalliferous compounds, such as sulfids, from the rock or earthy gangue with which 15 they are originally intermixed. More particularly, this invention relates to apparatus of the type commonly designated as "flotation," wherein pulverized ore, mixed with water and oily material, is agitated for the 20 separation of the metalliferous particles by taking advantage of their known preference for oily globules or bubbles.

For the efficient separation of metalliferous particles from the gangue by the flotation process, it is necessary that such particles be brought into intimate engagement 25 with the oily bubbles or globules. It has heretofore been proposed to effect such result by subjecting the pulp to agitation by paddle wheels submerged in the pulp. Such submerged paddle wheels, however, have necessitated a large expenditure of power, and have proved inefficient in that they have 30 been effective in aerating the pulp only by a occlusion of air or by drawing in air by a vortex formed by rapid rotation of the wheel. The resulting inefficient separation 35 of the metalliferous particles from the gangue has necessitated the use of apparatus comprising a number of units in which the 40 pulp is successively agitated, and the cost of installation and maintenance of such apparatus has limited the number of units, with the result that there has been an incomplete 45 separation of the metalliferous values from the gangue. To obviate this difficulty, it has also been suggested to run the paddle wheels only partly submerged and to substitute 50 drum agitators. While possessing certain economic advantages, these substituted agitators have failed to accomplish the end sought. It has also been proposed to effect 55 the agitation by the use of jets of compressed air. This type of agitation, however, has tended to produce a relatively small number of large bubbles with a result-

ing incomplete separation of the metalliferous values from the gangue.

It is an object of this invention to provide improved apparatus of the type stated 60 which, with the use of a less number of units, secures by agitation a thorough homogenizing of the frothed ore pulp and obtains a maximum separation of the metalliferous values from the gangue. 65

A further object of this invention is to provide a device of the type characterized wherein the agitator is not submerged in the ore pulp and therefore requires a minimum expenditure of energy to drive the same. 70

A still further object of this invention is to provide a device of the type described with an improved agitator whereby the ore pulp is thoroughly agitated without the production of large bubbles and the metalliferous values are separated and carried by a thick creamy froth having a low percentage of moisture. 75

Other objects relate to the provision of a device of the type characterized which is 80 simple in construction, inexpensive to manufacture, efficient in operation, and has a maximum capacity for the space occupied.

Stated broadly the invention comprises an agitating chamber, means for supplying 85 said chamber with ore pulp, preferably delivering said pulp to said chamber vertically, an agitator within said chamber and preferably closely fitting the same, and a settling chamber to which the agitated pulp 90 is delivered from the agitator. Said agitator, in its preferred construction, comprises a horizontal shaft supporting a series of plates inclined to the axis of said shaft and connected by interposing members 95 which may have the function of vanes in assisting in the agitation of the pulp. Means are also preferably provided for thoroughly aerating the pulp prior to its delivery to said agitating chamber, such means 100 being shown as a nozzle for introducing compressed air into the pulp as it rises through the conduit delivering to said chamber. Means are also preferably provided for the escape of air from the agitating chamber 105 prior to the delivery of the agitated pulp by the agitator to the settling chamber.

The invention is capable of receiving a variety of mechanical expressions, one of which is shown on the accompanying drawing, but it is to be expressly understood that the drawing is for purposes of illustration 110

only and is not to be construed as a definition of the limits of the invention, reference being had to the appended claims for that purpose.

5 In said drawing

Figure 1 is a plan view of a single-cell apparatus embodying the present invention, with the upper portion removed to more clearly illustrate the agitator; and

10 Fig. 2 is a vertical cross section through said apparatus.

Referring in detail to said drawing, wherein the same reference characters indicate corresponding parts in the several figures, 1 designates a suitable frame which supports, preferably adjacent the upper end thereof, an agitating chamber 2. Within chamber 2 is an agitator 3, shown as comprising a horizontal shaft 4 rotatable in suitable bearings 5 on the frame 1 and carrying a pulley 6, and a series of circular plates 8 mounted upon said shaft and slightly inclined with respect to the axis thereof. The plates 8 are maintained in parallel relationship by spacing collars 9 of any suitable material carried by said shaft and having their end faces inclined to said shaft at the same angle as said plates 8. To stiffen the plates 8 and maintain the same parallel, they 25 may be connected, adjacent their peripheries, by interposed members 10 suitably secured thereto. For convenience of construction, said members 10 may be constituted by longitudinal strips extending through each of the plates of the series and suitably riveted or soldered thereto. Any suitable number of these members 10 may be employed, and they may be made desirably of such shape and width as to constitute vanes and assist 30 in the agitation of the pulp delivered thereto. As shown, the members 10 are uniformly spaced circumferentially of the plates 8 and positioned in planes tangential to a relatively small circle concentric with the axis of the agitator 3 (see Fig. 2). To 35 prevent the ore pulp flowing longitudinally of the agitator, the latter is preferably made to closely fit the interior of the agitating chamber, and to this end the latter, if not circular in cross-section, is provided with longitudinal blocks or strips 11 interiorly shaped to conform with and closely envelop the periphery of said agitator.

Any suitable means may be provided for 40 supplying the agitating chamber with ore pulp. As shown, a vertical conduit 12 communicates at its upper end with said chamber and is supplied with ore pulp by any suitable feed pipe 13' adjacent the lower end 45 of said conduit. Means are also preferably provided within this conduit 12 to thoroughly aerate the pulp, and to this end compressed air is introduced into the upwardly flowing pulp through any suitable nozzle 13, preferably positioned adjacent the lower end

of the conduit 12. The compressed air so introduced into the pulp also assists in elevating the same to the agitating chamber and constitutes in effect an air-lift.

From the agitator the pulp is delivered to 50 a settling chamber 14, preferably provided with an inwardly inclined side or bottom 15 to guide the heavy particles settling therein toward the tailings-discharge pipe 16. By 55 preference, the agitated pulp is not thrown from the agitator onto the surface of the liquid in the settling chamber but is delivered thereto through a downwardly directed conduit 17 which extends to an appreciable distance below the surface of the liquid in 60 said chamber. Means are also preferably provided for the escape of air from the pulp prior to its delivery from the agitator to the settling chamber, and to this end an upwardly directed conduit 19 is in communication with the upper portion of the agitating chamber 2. For convenience of construction, conduits 17 and 19 may have a 65 common wall as shown at 18.

Any suitable means may be provided for 70 discharging the froth collected on the surface of the liquid in the settling chamber to any suitable launder (not shown), a paddle wheel 20 rotatable by any suitable means being diagrammatically illustrated on the 75 drawing.

In operation, the ore is ground and intermixed with water, and a suitable quantity of oil or similar substance, to provide a 80 pulp of the proper consistency. Said ore pulp is fed in any suitable way through pipe 13', as by gravity or pressure, into the lower end of the vertically directed conduit 12, in 85 which it rises to the settling chamber 2. In said conduit 12, the pulp is thoroughly aerated by compressed air admitted through nozzle 13 which assists also in the delivery of the pulp to said agitating chamber. The ore pulp is thrown from conduit 12 onto agitator 3, rotating in the direction of the 90 arrow shown in Fig. 2, by which it is carried around and discharged into conduit 17. Owing to the inclination of the plates 8, and aided by the vanes constituted by the interposed members 10 when used, the ore pulp 95 is slapped and beaten whereby large bubbles are broken up and the oil and air are intimately intermingled with the metalliferous particles. Much of the air is beaten out of the pulp during this operation and escapes 100 through the conduit 19. Owing to the close fit of the agitator within the agitating chamber, the pulp cannot flow longitudinally thereof but is carried around by the agitator and discharged into the conduit 17. The 105 frothy pulp discharged into the conduit 17 flows downwardly into the settling chamber, and the tiny globules or bubbles of oil-in-110 cased air, with the metalliferous particles adhering thereto, rise to the surface of the 115 pulp and are carried by the pulp into the 120 conduit 19. The pulp is then delivered into the settling chamber 14, where the heavy particles 125 settle and are carried by the inclined side or bottom 15 into the tailings-discharge pipe 16. The 130 pulp is then delivered into the settling chamber 14, where the heavy particles settle and are carried by the inclined side or bottom 15 into the tailings-discharge pipe 16.

liquid in the settling chamber and constitute a thick creamy froth having a relatively small proportion of moisture and air, and carrying a relatively large proportion of 5 metalliferous values. The heavier particles and the gangue sink to the bottom of the settling chamber 14 and are deflected laterally by the inclined side 15 toward the tailings-discharge pipe 16. The froth accumulated 10 on the surface of the liquid flows into the launder provided, aided by the paddle wheel when used.

Inasmuch as the agitator does not run immersed in the ore pulp, a relatively small 15 expenditure of power is sufficient to run the same, and, owing to the efficient aeration and agitation produced by the apparatus, with the consequent formation of a relatively large number of small bubbles or globules 20 intimately intermixed with the particles of ore pulp, an efficient separation of the metalliferous values from the gangue is obtained.

Some ores, however, are of such nature 25 that a single aeration and agitation of the same is insufficient to separate the metalliferous values therefrom. In such event, the apparatus may be constructed in the form of a plurality of cells, each preceding cell communicating with the vertical supply 30 conduit 12 of the succeeding unit and the last unit or cell being provided with a tailings-discharge pipe 16. Inasmuch as the type of agitator employed does not admit of a flow of the pulp longitudinally thereof, 35 an agitator may be provided for all of the units by extending the agitating chamber and the agitator itself throughout the length of the apparatus.

While the embodiment illustrated on the 40 drawing has been described with considerable particularity, it is to be understood that the invention is not to be limited to the precise structure shown but is capable of receiving a variety of mechanical expressions, 45 some of which will readily suggest them-

selves to those skilled in the art. Furthermore, certain features thereof are capable of use to the accomplishment of an improved result without the use of other features thereof. Reference is therefore to be had 50 to the appended claims for a definition of the limits of this invention.

What is claimed is:

1. In flotation apparatus, the combination of a vertical conduit, means for introducing 55 at the base of said conduit ore pulp and a jet of air to produce an upwardly flowing column of frothed pulp, a chamber located at the top of said conduit for receiving said frothed pulp, froth beating means in said 60 chamber adapted to beat said frothed pulp as led into the froth beating chamber, a froth separating tank and a conduit open to said chamber and having one end opening into the atmosphere for venting of air and 65 the opposite end delivering froth to said tank.

2. In combination, a froth separator, a beater, an uprising conduit adapted to feed a body of commingled ore pulp and gas 70 bubbles directly to said beater, said beater adapted to beat the whole of said pulp into a froth and deliver the same to said froth separator.

3. In a flotation process for treatment of 75 ore pulp which consists of a mixture of ore in fine division, water and a frothing agent, the steps consisting in injecting air into an upwardly moving column of said pulp to produce a body of froth at the top of said 80 column, beating the froth in a confined space at the top of the column as it leaves said column to break up the larger air bubbles and produce a creamy froth while permitting excess of air to escape, and then separating 85 the froth and gangue.

In testimony whereof I have signed this specification.

WILLIAM L. ZIEGLER.